

June 6, 1933.

R. H. V. CHRISTENSEN ET AL

1,913,071

APPARATUS FOR POURING MELTED METAL UNDER PRESSURE

Filed Jan. 2, 1931

2 Sheets-Sheet 1



Inventors

Reinhardt Harald Valdemar  
Christensen  
and Richard Smith Dahl  
By Dowell & Dowell  
Attorneys

June 6, 1933.

R. H. V. CHRISTENSEN ET AL

1,913,071

APPARATUS FOR POURING MELTED METAL UNDER PRESSURE

Filed Jan. 2, 1931

2 Sheets-Sheet 2



Inventors  
Reinhardt Harald Valdemar  
Christensen  
and Richard Smith Dahl  
By Dowell Ed Dowell  
Attorneys

## UNITED STATES PATENT OFFICE

REINHARDT HARALD VALDEMAR CHRISTENSEN, OF COPENHAGEN, AND RICHARD SMITH DAHL, OF GENTOFTE, DENMARK

## APPARATUS FOR POURING MELTED METAL UNDER PRESSURE

Application filed January 2, 1931, Serial No. 506,280, and in Denmark January 7, 1930.

This invention aims to provide an improved process and apparatus for pouring molten metal, such as iron, phosphor-bronze and aluminium under pressure.

5 In castings of this nature it is known to withdraw the molten metal from the crucible by means of a pouring ladle, which is then connected to the mould. The process according to the present invention is distinguished 10 from this in that the metal is transferred from the ladle to the mould by the creation in the mould of a relatively low differential pressure, for instance a vacuum, that the inlet of the mould is then closed, and that 15 the metal enclosed in the mould is then exposed to a pressure. According to the invention the vacuum in the mould may be produced by the air in the mould being sucked out at several points.

20 The apparatus according to the invention is partly characterized in that a portion of the inlet of the mould is formed by a cylindrical channel adapted to receive a piston, which piston, when moved forward towards 25 the mould cavity, first closes the connection to the latter and then exerts a pressure on the enclosed metal. Other distinguishing features of the apparatus will appear from the following description of various practicable embodiments of the invention as 30 shown in the drawings, wherein

Fig. 1 illustrates a casting machine, in side elevation, partly in section,

Fig. 2 is a top view of the same,

Fig. 3 illustrates another constructional form of casting machine in side elevation, partly in section; and

Fig. 4 is a cross-section of the latter on the line IV-IV of Fig. 3, showing associated valve mechanism employed in both constructions.

The casting machine shown in Figs. 1 and 2 embodies a frame 10 fitted at the ends with brackets 11 interconnected by round bars 12 serving as guide bars. Two holding plates 13 and a holding member 14 are adapted to slide on these bars, and the member 14 is adjustably connected to one of the holding plates 13 by means of threaded sleeves 15 provided on the bars 12. The parts 16

of the mould are connected to or between the holding plates 13 in such positions that the mould parts will engage one another correctly, when the holding plates are drawn toward one another. In one of the brackets 11 a shaft 17 is journaled, which shaft supports two toothed segments 18 engaged by pinions 19, which are mounted on another shaft 20 journaled in the same bracket and actuated at one end by a capstan wheel 21. Arms 22, integral with the segments 18, together with length-adjustable link members 23 form knee-presses adapted to actuate the holding member 14 when the capstan 21 is rotated.

At one end of the casting machine a furnace 24 is provided containing a crucible 25, in which the casting material is heated.

The transfer of the molten metal to the mould 16 is effected by a pouring ladle 26 which in the present instance is made of a refractory material shaped like a block and having a mainly U-shaped channel 27 adapted to hold the mould charge. This ladle is suspended with free pivoting on a crank 27', the shaft 28 of which is journaled in a bracket 29 attached to one of the brackets 11 and adapted to be actuated by means of a crank handle 30. For transferring the ladle from the crucible to the mould, the shaft 28 is turned through an angle of 270° by the handle 30, whereafter the ladle will be in the position shown in Fig. 1. In this position, one orifice of the channel 27 communicates with the inlet 31 of the mould by way of a refractory lining 32 inserted in one of the holding plates 13. The other orifice of the channel 27 communicates with the atmosphere by way of a sleeve 33 forming a resilient support for the ladle 26, as the sleeve 33 is adapted to slide in the above mentioned bracket 11, counteracted by a spring 34. When the pouring ladle is situated in the above mentioned position, then the mould parts 16 are moved together by means of the aforescribed knee-presses 22, 23 actuated by the capstan 21. When the mould parts have come into contact with one another, they are moved together a short distance by further rotation of the capstan,

100

until the front holding plate 13 strikes a suitable stop. During this last motion the ladle 26 is pressed firmly between the lining 32 and the sleeve 33 under a pressure determined by the tension of the spring 34. By this means it is assured that the ladle 26 will not be subjected to excessive lateral pressures or stresses.

- 10 The liquid metal taken up in the channel 27 of the ladle is drawn into the cavity 35 of the mould by a vacuum created in the latter. From the mould cavity a channel 36 extends, which at the start is situated in the dividing surface between the mould 15 parts, i. e. half of the channel is worked into each mould part, and then the channel is continued in the foremost mould part 16 (situated next to the furnace 24). From the channel 36 extends a flexible pipe 37, which 20 by way of a valve 38 leads to a suction pump (not shown).

If desired, the liquid metal may also be transferred to the mould by supplying compressed air, at a relatively low pressure to 25 the sleeve 33 on the other side of the ladle 26.

A portion of the inlet of the mould is formed by a cylindrical channel 38' adapted to receive a rod-like plunger 39, which latter, 30 when moved forward towards the mould cavity 35, first cuts off the connection from the pouring ladle 26 to said cavity, and then exerts a pressure on the enclosed metal. The axis of the plunger 39 is mainly situated 35 in the dividing plane of the mould, in such a manner that the solidified plug of metal below the plunger can be removed together with the dead head in the inlet, when the mould parts are separated at the removal of 40 the casting.

The plunger 39 supports at its extreme end a disc 40 forming the piston for a cylinder 41, to the top part of which compressed air can be supplied by way of a 45 valve 42 and a pipe 43 from a not shown source of compressed air, when said piston is to be moved inward. The cylinder 41 is supported by a bracket 44 attached to the front holding plate 13, so that the cylinder 50 is always in firm connection with the foremost mould part 16. The piston 39 will therefore continue to be in contact with this mould part, when the other mould part is withdrawn during removal of the casting. 55 To the rear holding plate 13 there is attached an arm 45, the extreme bent end of which co-operates with a stop 46 on the plunger 39, when the said holding plate is moved back, so that the plunger is automatically returned to the initial position 60 when the mould is opened.

The valves 38 and 42 are conveniently mounted in a bracket 70 affixed to the front holding plate or frame, with the first-named 65 (38) thereof controlling a connection of the

pipe 37 with a pipe 72 leading to the aforementioned suction pump and the second-named (42) controlling a connection of the pipe 43 with a pipe 71 leading from the aforesaid source of compressed air. These 70 valves, as best shown in Fig. 4, are advantageously controlled by a common device, which in the illustrative example is formed by a two-armed lever 47, which is pivoted on a pin 48 and one arm of which co-operates with the spindles of the valves, while the other arm is adapted to be actuated from the rear end of the casting machine by a cord or chain 49. By this arrangement the advantage is attained that the two valves are always operated in proper succession, the valve 38 being opened first and then the valve 42.

It should be noted that the first part of the exhaust channel 36 is so narrow that the melted metal will solidify from cooling against the form parts 16 before passing any appreciable distance into this channel, which will therefore become clogged. Accordingly, the melted metal cannot possibly be sucked out through the pipe 37.

The modification or construction of the casting machine shown in Figs. 3 and 4 will now be described in so far as it differs from that just described.

In this machine there is inserted, between the rear holding plate 13 and the mold part 16 supported by the same, a supporting member 51, whereby space is provided for a not shown mechanism serving to withdraw any cores used in connection with the mould. The front holding plate 13 is stationary, and is constructed as a bracket attached directly to the frame 10.

The melted metal is supplied to the mould by way of an angular inlet pipe 52 made preferably from refractory material. This pipe is placed in such manner that one branch thereof is vertical and the other one horizontal. The horizontal branch passes air-tight through the front holding plate 13, against which the corresponding mould part 16 is pressed air-tightly, and ends at a cavity 53 in the mould, from which cavity the inlet proper 54 to the cavity 35 of the mould extends. The outlet orifice from the horizontal branch opens to the inlet 54. The inlet orifice at the free end of the vertical branch is situated relatively close to the surface of the liquid metal in the crucible 25. In this case the pouring ladle is movable in vertical direction and serves to transfer definite quantities of the liquid metal from the crucible to the said inlet orifice. The said ladle is formed as a vertical pipe 56 of refractory material closed at bottom and encircling the vertical branch of the pipe 52. The pipe 56 is formed on one side with a slit 57 for the horizontal branch of the inlet pipe and, along a horizontal plane some 115 120 125 130

distance above the bottom, one or more openings 58 determining the top level of the quantity of metal contained in the pipe.

The pipe 56 is suspended on a mechanical moving device actuated automatically by the motion of the movable mould part. This mechanical device is formed by a bell-crank lever 59 pivoted on a pin 60 on the front holding plate 13. The one horizontal arm 10 of the lever is connected to the pipe 56 by means of a link member 61. The end of the other arm of the lever is fitted with an adjustably disposed screw 62, the end of which is adapted to co-operate with the rear mould 16, when the latter is in vicinity of the front mould part. The screw 62 can be adjusted in such a manner that by the motion of the movable mould part towards the stationary mould part the pipe 56 will be raised 20 to such a level that just one mould charge will be taken up to be transferred from this pipe to the inlet pipe 52 by suction through the last mentioned pipe. The distance between the liquid level in the raised pipe 56 25 and the downward facing orifice of the pipe 52 is in fact the feature determining the quantity of metal to be transferred to the mould, because when the liquid level reaches the said orifice the intake of metal will cease, 30 whereafter only the column of metal contained in the pipe 52 will be conveyed to the mould owing to its kinetic energy.

In this modified construction as shown in Fig. 4, the piston 39 and the cylinder 41 are 35 disposed in sloping manner, in order to provide space for the end of the pipe 52 situated in the cavity 53.

The channel by way of which the mould is evacuated is in this case ramified and connected to the mould cavity 35 at several 40 points. Hereby any accumulation of air in the mould during the pouring will be avoided, and the effect of any leaks will be eliminated. The ramification is effected by cutting furrows or grooves 63 in the contacting surfaces of the mould parts, which grooves when the mould parts are placed together form a channel, which encircles all the cavities of the mould, and from where 45 branches 64 extend to the said cavities. The annular channel is connected to the suction line 37 by way of the channel 36 in the front stationary mould part 16.

The machine is otherwise constructed in 50 similar manner to that first described, and the corresponding parts in the two machines are marked with the same reference numerals.

In this construction of the machine the 55 liquid metal transferred by way of the pipe 52 will first be received by the cavity 53, which is sufficiently large to hold the entire mould charge. From this cavity the metal is conveyed to the mould cavity, mainly by 60 action of gravity alone.

The here described constructions may be modified in various respects without deviation from the essential features of the invention. Thus the piston which limits the mould charge received by the mould and exerts a pressure thereon may be moved by purely mechanical means, such as a screw or the like, instead of the valve mechanism shown and described in detail with reference to Figs. 1 and 2.

The advantage of the process according to the present invention is not only that alloys and metals with high melting point and being difficult to pour can be cast, but also denser and more uniform castings are attained than according to the here known squirming method of casting, according to which a metal superheated above the fusing point is flung forcefully into the mould. By this last mentioned casting method the introduction of the metal is so violent that it is flung against the walls of the mould in such a manner that at certain points the air in the mould may become enclosed, while the metal, where the wall is thin, may become solidified before the entire pouring is finished, the consequence being that the advantages of the pressure used cannot manifest themselves. The castings will therefore be porous and less uniform, and may contain air blisters. These drawbacks may certainly be avoided by another known casting method, i. e., the so-called chill casting, which method, however, is not suited for mass-production and does not give so fine and sharp castings as does the squirming method.

A distinguishing feature of the process according to the present method is that the metal is introduced into the mould by a relatively low differential pressure, so that the conditions will be approximately the same as if the metal were poured into the mould, and that the metal is then exposed to a considerable pressure, so that it will fill the mould entirely. The use of a high pressure on the metal, after the same is introduced into the mould, is mainly rendered practicable by the feature that the pressure does not act on the ladle.

Having now particularly described and ascertained the nature of our invention and in what manner the same is to be performed we declare that what we claim is:

1. In an apparatus for casting metal under pressure, a mould, a ladle adapted to receive molten metal and to be subsequently connected with the mould, an inlet channel in the body of the mould arranged to communicate with the ladle when the latter is connected with the mould and situated above the mould cavity so as to allow the molten metal to be transferred against the action of gravity from the ladle to said inlet channel and to fill the mould cavity by gravity,

- a second channel situated in the body of the mould and communicating with said inlet channel, and a plunger arranged to advance in said channel so as to cut off the flow of the molten metal from the ladle to the inlet channel and to subsequently subject the metal in the mould to pressure.
2. An apparatus for casting metal under pressure, comprising a mould formed in two parts, an inlet channel for molten metal disposed in the body of the mould above the mould cavity, a ladle adapted to receive molten metal and to be connected with the mould so as to communicate with said inlet channel of the latter by an upwardly disposed passage through which the metal may be transferred from the one to the other against gravity action, a channel formed by the two parts of the mould and communicating with said inlet channel, and a plunger arranged to advance in the last-named channel so as to cut off the flow of the molten metal from the ladle to the mould and to thereafter subject the metal in the mould to pressure.
3. An apparatus for casting molten metal under pressure, comprising a mould formed in two parts, an inlet channel in one part of the mould above the mould cavity, a channel formed by the two parts of the mould in communication with said inlet channel, a ladle adapted to receive molten metal and to be connected with the mould, communicating passages with means for forcing the molten metal from the ladle into said inlet channel against gravity action and to allow the molten metal thereafter to fill the mould cavity by gravity, a plunger located in the second-named channel, and means for advancing the plunger in said second-named channel so as to first cut off the molten metal supply from the ladle to the mould and then subject the molten metal within the mould to pressure.
4. An apparatus for casting molten metal under pressure, comprising a mould formed in two parts, an inlet channel in one of said parts at a level higher than the mould cavity, another channel formed in the two parts of the mould and communicating with said inlet channel, a ladle adapted to receive molten metal and to be connected with the mould in an upward passage communication with said inlet channel thereof, an evacuating channel in the mould body communicating with said mould cavity and therethrough with said inlet channel, means for creating a vacuum in the mould through the evacuating channel to draw the molten metal from the ladle into the inlet channel of the mould against gravity action and allowing the metal to flow from said inlet channel into the mould by gravity, means for interrupting the vacuum action, a plunger working in the second-named channel, and means for moving said plunger to first cut off the supply of molten metal from the ladle to the inlet channel and then to subject the molten metal in the mould cavity to pressure.
5. An apparatus for casting molten metal under pressure, comprising a mould formed in two parts, an inlet channel in one of said parts at a level higher than the mould cavity, a cylindrical channel formed by the two parts of the mould and communicating with said inlet, a ladle adapted to receive molten metal and to be connected with the inlet of the mould through an upwardly directed passage, an evacuating channel in the mould body communicating with the mould cavity, means for creating a suction through said evacuating channel to draw the molten metal against gravity action from the ladle into the inlet channel of the mould and allowing the metal to flow from said channel into the mould by gravity, a plunger working in the cylindrical channel, means for interrupting the suction action and means for moving said plunger to first cut off the flow of metal from the ladle to the inlet channel and then to subject the molten metal in and flowing to the mould cavity from the inlet channel by gravity to pressure.
6. An apparatus for casting molten metal under pressure, comprising a mould formed in two parts, an inlet channel in the body of the mould above the mould cavity, an angular inlet pipe projecting into said inlet channel through an airtight seal, a ladle encircling the lower end of a downwardly directed portion of said inlet pipe and arranged to receive predetermined amounts of molten metal, means for adjusting the ladle vertically to cause the molten metal therein to surround the lower end of said pipe portion, an evacuating channel in the mould body communicating with the cavity of the mould, means for creating a suction in the mould through said evacuating channel to draw the metal through said inlet pipe from the ladle to the inlet channel of the mould, a cylindrical channel formed by the two parts of the mould in communication with the inlet channel, a plunger working in said cylindrical channel, means for interrupting the suction action in the mould when sufficient molten metal has been drawn thereinto, and means for thereafter causing the plunger in the cylindrical channel to advance to first cut off the supply of metal through the inlet tube and then to subject the metal drawn into the mould to pressure.
7. An apparatus for casting molten metal under pressure, comprising a mould formed in two parts, an inlet channel in the body of the mould above the mould cavity, an angular inlet pipe projecting into said inlet channel through an airtight seal, a ladle en-

circling the lower end of a downwardly directed portion of said inlet pipe and arranged to receive predetermined quantities of molten metal, means for adjusting the 5 ladle vertically to bring the molten metal therein around the lower end of said pipe portion, an evacuating channel in the mould body in communication with the mould cavity, means for creating a suction in the 10 mould through said evacuating channel to draw the metal from the ladle through the inlet pipe to the inlet channel of the mould, a cylindrical channel formed by the two parts of the mould in communication with 15 the inlet channel, a plunger working in said cylindrical channel, means for interrupting the suction action in the mould when sufficient of the molten metal has been drawn thereinto and means for thereafter causing 20 the aforesaid plunger in the cylindrical channel to advance to first close the connection between the angular tube and the mould cavity and to then subject the metal in the latter to pressure.

25 8. An apparatus for casting metal under pressure, comprising a mould formed in two parts of which one is stationary, means for moving the other part to and from the stationary part, a ladle adapted to receive 30 molten metal and movable automatically in cooperation with the aforesaid means to a predetermined raised position when the mould parts are brought together, an inlet channel in the mould, an angular pipe having 35 one branch fitted airtight in the inlet channel of the mould and the other branch extended downwardly into the lower end of the ladle, an evacuating channel in the mould body communicating with the cavity of the mould, means for creating a suction in the mould through said evacuating channel to draw the metal from the ladle through the angular pipe to the inlet channel of the mould, a cylindrical channel 40 formed by the two parts of the mould in communication with the inlet channel, a plunger working in said cylindrical channel, means for interrupting the suction in the mould when sufficient molten metal has been 45 drawn thereinto, and means for thereafter causing said plunger to advance in its cylindrical channel to cut off the molten metal flow from the ladle to the mould cavity and to then subject the metal in the mould to 50 pressure.

55 REINHARDT HARALD VALDEMAR CHRISTENSEN.  
RICHARD SMITH DAHL.